

H. DEDICHEN & O. HALSE.

PROCESS OF REFINING AND DEODORIZING RAW TURPENTINE OILS.

APPLICATION FILED JAN. 31, 1917.

1,253,793.

Patented Jan. 15, 1918.

Fig.2.

Fig.1.



Inventors:  
Herman Dedichen  
Ole Halse  
By Henry Orth Atty.

# UNITED STATES PATENT OFFICE.

HERMAN DEDICHEN AND OLE HALSE, OF CHRISTIANIA, NORWAY, ASSIGNEES TO  
UNION CO., OF CHRISTIANIA, NORWAY.

## PROCESS OF REFINING AND DEODORIZING RAW TURPENTINE-OILS.

1,253,793.

Specification of Letters Patent. Patented Jan. 15, 1918.

Application filed January 31, 1917. Serial No. 145,757.

To all whom it may concern:

Be it known that we, HERMAN DEDICHEN and OLE HALSE, both subjects of the King of Norway, and residing at Christiania, in the 5 Kingdom of Norway, have invented certain new and useful Improvements in the Processes of Refining and Deodorizing Raw Turpentine-Oils; and we do hereby declare the following to be a full, clear, and exact 10 description of the invention, such as will enable others skilled in the art to which it appertains to make and use the same.

Our invention relates to the treatment of crude turpentine oils and more particularly 15 to a process for deodorizing such oils especially turpentine oils which are obtained as a byproduct in the manufacture of cellulose according to the soda cellulose process.

It is a matter of fact that such turpentine 20 oil has a very disagreeable odor which is supposed to be caused by organic sulfur compounds, and that this odor has prevented the utilization of these oils to any considerable extent, the oils having also 25 proved unsuitable for medical use.

Several methods have been tried to remove the said compounds by submitting the 30 oils to a repeated distillation but without success. It has also been proposed to destroy the odorous matter by chemical means for instance by means of nitrous gases or ozone, or to precipitate it by means of mercury chlorid, but such processes have been without practical result.

35 Further it is known that such oils are improved when exposed to daylight and the action of air for a long time but to use such method in the manufacture has proved impossible because the treatment in order to 40 obtain any kind of useful result must take a long time in fact two years and more.

Our invention now consists in a process 45 for deodorizing said oils by the action of active rays and an oxidizing agent, and more especially it is based upon the observation 50 that when crude bad smelling turpentine oil is exposed to the action of very strong or active light, the oil is in a short time so improved as to its odor that it is possible to produce a marketable turpentine oil in this manner. We have found that for 55 the purpose of our invention we can with great advantage make use of ultra violet light, Röntgen rays, dark electric discharges and the like.

In carrying out our invention the desired result may be obtained in various ways, for instance by submerging a source of chemically active rays in the oil while blowing an oxidizing gas through the oil but, we 60 have found it preferable to treat the raw oil in a state of dispersion with chemical active rays as for instance ultra violet light. After a comparatively short time the disagreeable odor disappears and a product is obtained, 65 which we may submit to a usual steam distillation, whereby a transparent and colorless oil is obtained, which in all respects is like the usual American turpentine oils. It is preferable that the oil be exposed to the 70 action of air or oxygen during the treatment.

The invention may be carried out by causing the raw oil to flow slowly in very thin layer down a slightly inclined surface, 75 which preferably should be white, being thereunder exposed to the air and to the action of light emitting from a usual quartz-mercury lamp. After a comparatively short exposure to the light the oil becomes odorless and when afterward distilled by steam 80 it becomes transparent and colorless.

An apparatus for carrying this process into effect is diagrammatically illustrated in the accompanying drawing in which— 85

Figure 1 is a side view of the apparatus, and

Fig. 2 is a front view of the same.

In the illustrated example, 1 designates a glass plate the back of which is provided 90 with a white coating 2. Glass rods 3 are arranged across the surface of the plate 1 to prevent a too rapid flow of the liquid down said plate. The raw turpentine oil is supplied through pipes 5 at the upper end of 95 the plate and the refined oil flows through the funnel 6 into the container 7 from which the oil, if necessary, may be drawn off at 8 and by means of pumps (not shown) supplied to the pipes 5 for repeated treatment. 100 A mercury lamp 9 is arranged above the plate 1.

The same good result may also be obtained by treating the oil vaporized or in diffused or similarly finely divided form by 105 chemical active rays, preferably in the presence of air, oxygen or other suitable gases, which may be caused to pass the zone of active light in the same or in the opposed direction of the oils.

We have found by way of a very careful fractional distillation and determination of physical constants as for instance specific gravity, rotation capacity, index of refraction and molecular refraction that the product obtained according to our process consists of about  $\frac{2}{3}$   $\alpha$  pinene and  $\frac{1}{3}$   $\beta$  pinene. As is well known the usual French and American turpentine oils have the same constitution.

From the usual turpentine oils the product obtained according to the present invention differs therein that it contains dextrorotatory  $\beta$  pinene, while the  $\beta$  pinene contained in the ordinary products is of the levo-rotary modification.

In some cases, especially when the oils are very bad smelling, it is preferable to remove the greater part of the smelling substances, before the oils are exposed to the light process, by treating them with a non-gaseous oxidizing agent such as chlorid of iron, copper or zinc or a mixture of these salts; simultaneously air may be driven through the oil. The oil may also be treated in this manner after exposing it to the light process if after the latter there remain traces of unpleasant odor. This process can be performed in the simplest manner by shaking the oil with small quantities of a concentrated solution of the said salts in water, alcohol or other suitable solvent. The operation can be carried out at usual temperature or at a slightly raised temperature and can be supported by supplying air to the liquid.

We claim:

1. In the process of refining and deodorizing raw turpentine oils the step which consists in exposing the raw oil to the action of chemically active rays in the presence of an oxidizing agent.
2. The process which consists in subjecting raw turpentine oil obtained as a by-product in the soda cellulose process, to the action of ultra violet rays in the presence of an oxidizing agent.
3. In the process of refining and deodor-

izing raw turpentine oils the step which consists in exposing the raw oil to the action of chemically active rays in the presence of an oxidizing agent in a state of dispersion.

4. The process which consists in dispersing raw turpentine oil and causing it to move in a dispersed condition through a zone of chemically active rays in the presence of an oxidizing gas.

5. The process of refining and deodorizing raw turpentine oil which comprises the operations of subjecting the oil to the action of chemically active rays in the presence of a gaseous oxidizing agent, and of treating the oil with a non-gaseous oxidizing agent, the oil being first subjected to one and then to the other of the said operations.

6. The process of refining and deodorizing raw turpentine oil comprising the operations of subjecting the oil to the action of chemically active rays in the presence of a gaseous oxidizing agent, and of treating the oil with a non-gaseous oxidizing agent, the oil being first subjected to one and then to the other of the said operations whereupon the oil is submitted to a distillation process.

7. The process of refining and deodorizing raw turpentine oil comprising the operations of subjecting the oil to the action of chemically active rays in the presence of a gaseous oxidizing agent, and of treating the oil with chlorid of iron, the oil being first subjected to one and then to the other of the said operations.

8. As a new product of manufacture a refined turpentine oil consisting of a pure mixture of  $\alpha$  pinene and  $\beta$  pinene and comprising dextro-rotatory  $\beta$  pinene.

In testimony that we claim the foregoing as our invention, we have signed our names in presence of two subscribing witnesses.

HERMAN DEDICHEN.  
OLE HALSE.

Witnesses:

C. VARMAN,  
THS. BERG.